

## UNITED STATES PATENT OFFICE.

LOUIS HIPPOLYTE ERNEST LACROIX, OF PONT DE CHÉRUY, FRANCE,  
ASSIGNOR TO JOSEPH LOUIS ROUTIN AND LÉON MARTIAL EUGENE  
MOURRAILLE, OF LYONS, FRANCE.

## METALLIC ALLOY.

SPECIFICATION forming part of Letters Patent No. 782,401, dated February 14, 1905.

Application filed May 14, 1904. Serial No. 207,897.

*To all whom it may concern:*

Be it known that I, LOUIS HIPPOLYTE ERNEST LACROIX, a citizen of the French Republic, residing at Pont de Chéruy, Isère, France, 5 have invented a certain new or Improved Metallic Alloy, of which the following is a specification.

This invention relates to a new or improved metallic alloy, the purpose of which is to 10 serve as a substitute for lead for most of the purposes for which the latter is used.

This alloy is of greater strength and ductility than lead and is equally malleable.

The base of the alloy is lead; but the thickness of metal required for given purposes when the alloy is used is from twenty-five to forty per cent. less than that required when ordinary lead is employed, so that the weight of alloy which has to be used for any given 20 purpose is always considerably less than the weight of lead which would be necessary for the same purpose.

The components of the improved alloy are lead, antimony, and sodium in the following 25 proportions: lead, one thousand parts, by weight; antimony, fifteen parts, by weight; sodium, one part, by weight. These proportions produce an alloy having in the highest degree the advantages hereinafter stated; but 30 the proportions of antimony, sodium, and, consequently, the properties of the alloy can be varied according to the purpose for which the material is intended. The hardness of the alloy can, for instance, be increased by 35 increasing by suitable degrees the proportions of antimony and sodium, which may reach five hundredths, by weight, in the case of the antimony, and five thousandths, by weight, in the case of the sodium.

40 The alloy can be manufactured in different ways. The desired quantity of antimony can, for instance, be placed in a crucible and fused, whereupon the desired proportion of lead is added. When the mixture is fused, 45 the sodium is added and the whole is energetically agitated and then immediately poured out. The alloy of antimony and sodium can also be effected in one crucible, while the lead

is fused in a separate crucible. When the 50 contents of both crucibles are fused, the antimony and sodium are poured into the crucible containing the lead, whereupon the whole is energetically agitated and immediately poured out.

Very considerable direct economy is effected 55 by the use of the improved alloy, and the reduction of weight also has other advantages. Thus, for instance, if the new alloy is used for roofing in place of lead the beams and other parts of the structure can be made 60 lighter. The alloy is more easy to treat than lead and can be rolled into exceedingly thin sheets and drawn into very fine wire. The alloy is also more easy to solder than lead. It can, in fact, be soldered by means of an 65 ordinary soldering-iron without the use of a blowpipe. Like lead, the alloy is not attacked by nitric acid, sulfuric acid of 50° Baumé, sulfuric acid of 50° Baumé with nitrous gas, sulfuric acid of 66° Baumé, the 70 hydrochloric acid of commerce, distilled water, river - water, ten-per-cent. solutions of sea-salt, caustic soda of 25° Baumé, and so on. The alloy offers, generally speaking, 75 double the mechanical resistance of lead. Its coefficient of extension varies between twenty and thirty per cent. It can be worked in the lead-press to produce pipes which are size for size capable of resisting twice as great pressure as lead pipes.

I claim—

1. A metallic alloy consisting of lead, antimony, and sodium, the lead being in excess of the antimony and the latter in excess of the sodium.

2. A metallic alloy consisting of one thousand parts by weight of lead, fifteen parts by weight of antimony and one part by weight of sodium.

In witness whereof I have signed this specification in the presence of two witnesses.

LOUIS HIPPOLYTE ERNEST LACROIX.

Witnesses:

THOS. N. BROWNE,  
MARIN VACHORY.